

## UNITED STATES PATENT OFFICE.

YUJI SHIBATA, OF TOKYO FU, AND YUSHICHI NISHIZAWA, OF TOKYO, JAPAN.

## PROCESS OF DRYING JAPANESE LACQUER.

No Drawing.

Application filed March 29, 1920. Serial No. 369,792.

*To all whom it may concern:*

Be it known that we, YUJI SHIBATA and YUSHICHI NISHIZAWA, subjects of Japan, and residing, respectively, at No. 317 Hiya-kunincho, Okubo Machi, Toyotama Gun, Tokyo Fu, and at No. 110 Hakusan Goten Machi, Koishikawa Ku, Tokyo, Japan, have invented new and useful Improvements in a Process of Drying Japanese Lacquer, of which the following is a specification.

This invention relates to a process for drying Japanese lacquer, and consists in the addition to the lacquer preparation, of complex salts of certain metals. The object of this invention is to quicken the drying and hardening of lacquer coating and at the same time to prevent its surface from getting wrinkled.

Lacquer has been for a long time a special product of the Orient and as a varnish has many merits unrivalled by any other known substance. It has however some drawbacks, and is sometimes liable to collect irregularly, which impairs its appearance. Besides, a special equipment is necessary to accelerate its drying by supplying thereto sufficient heat and moisture. Thus, it is very difficult to apply this substance to any large surface such as a building or any article of considerable dimensions.

Now, while carrying on researches with regard to complex salts of certain metals, we have discovered a process by which the above drawbacks can be removed.

Our process consists in mixing one or more complex salts of copper and zinc, such as copper ammonic sulphate and zinc-ammonic sulphate, and complex salts cobalt, nickel, manganese, magnesium, calcium, tin and aluminium with a lacquer preparation in the proportion of from 5 to 10 per cent, and the result is that the coating made with the mixture dries so rapidly that what would take twenty-four hours to dry if treated according to a process hitherto known, will be effected in a few hours; and if the proportion of the complex salts of metals be increased to 20 or 30 per cent, the mixture will become plastic, and perfectly dry in an hour or two. This great rapidity with

which lacquer coating can be made dry, enables us to apply the substance to buildings, carriages, and any other large surface; and in this respect this invention considerably enlarges the sphere of usefulness of lacquer, to an extent which has never been attained before.

Of course lacquer is much more expensive than ordinary oil paint, but it is more durable and presents a more pleasing appearance too, and will last at least three times longer than the latter. Thus, in the long run, lacquer will prove cheaper coating material than paint.

The quick drying of lacquer brought about by our invention also prevents the coated surface getting wrinkled when drying. The reason why wrinkles are not produced is because there is no difference in viscosity according to our invention caused between the outer surface exposed to the air and inner part owing to oxydation, or drying, taking place more actively in the former than in the latter. Moreover, when a larger proportion of the complex salts of metals is added to lacquer preparation, not only does it quicken the hardening thereof, but gives thereto a certain degree of consistency. Further, our invention gives to lacquer greater viscosity, luster and covering power.

We claim:

1. A process of drying Japanese lacquer characterized by the admixture therewith of complex salt of a metal and ammonium, substantially as and for the purposes hereinbefore set forth.

2. A process of drying Japanese lacquer characterized by the admixture therewith of complex salts of copper ammonic sulphate, substantially as and for the purposes hereinbefore set forth.

3. An article of manufacture, comprising a Japanese lacquer preparation having therein a complex salt of metals and ammonium in the proportion of five to thirty per cent.

In testimony whereof we have signed our names to this specification.

YUJI SHIBATA.  
YUSHICHI NISHIZAWA.